

## UNITED STATES PATENT OFFICE

1,934,440

PROCESS OF CONCENTRATING ORE BY  
FLOTATION

Frederick G. Moses, New York, Raymond W. Hess, Buffalo, and Robert L. Perkins, East Aurora, N. Y., assignors to The Barrett Company, New York, N. Y., a corporation of New Jersey

No Drawing. Application February 15, 1927  
Serial No. 168,465

12 Claims. (Cl. 209—166)

This invention relates to the separation of minerals and the concentration of ores by flotation processes, and is particularly directed to such separation and concentration carried out with the utilization of certain organic sulfur compounds as flotation agents.

According to the present invention, the separation of minerals and the concentration of ores by the flotation operation is carried out with the aid of a carbocyclic mercaptan of the aromatic series which contains no nitrogen in its composition. The invention enables improved results to be obtained, these being manifested sometimes in better recoveries, sometimes in producing a higher grade concentrate, sometimes in reducing the time required for carrying out the flotation operation, and sometimes in effecting the usual recoveries with a lesser quantity of frothing agent than ordinarily required.

The aromatic carbocyclic mercaptans or thiophenols employed as the flotation agents or adjuvants in the process of the present invention comprise those nitrogen-free mercaptans which contains a mercapto group, —SH, bound or attached to a carbon atom which is a component member of an aromatic carbocyclic ring or nucleus (a nuclear carbon atom). They include the nitrogen-free mercaptans of the benzene, the naphthalene, the anthracene, and other aromatic carbocyclic series. Aromatic carbocyclic mercaptans of the benzene series are particularly important.

In general, the carbocyclic mercaptans or thiophenols employed in the present invention may be prepared by reducing an aromatic sulfonyl chloride, or by the action of an alkali hydrosulfide on a salt of an aromatic sulfonic acid, or by the action of an alkali metal sulfide or sulfhydrate, or a salt of xanthic acid, on an aromatic diazo compound. Other suitable methods may be employed. The pure or purified thiophenol body is preferably employed.

In carrying out the flotation process, the flotation agent comprising the nitrogen-free aromatic carbocyclic mercaptan body may be incorporated with the ore or the mineral pulp in any suitable manner and at any suitable time in accordance with customary known practices as will insure a satisfactory flotation operation. For example, it may be introduced in the free state or as a salt into the mill in which the ore is being ground, or it may be dissolved, suspended or dispersed in any suitable solvent or dispersing agent as, for example, in one or more of the usual flotation oils or oil mixtures, or in water or in an alkali

or alkaline reagent, and incorporating the resulting suspension, solution or dispersion with the ore or the ore pulp. While the agents of the present invention show marked action as flotation agents in ore concentration, they possess little, if any, frothing qualities and therefore are used to advantage in conjunction with any suitable or well known frothing agent, e. g. pine oil, crude turpentine, tar acids, etc. They may be also sometimes used to advantage in conjunction with other flotation agents.

The process of the present invention can be carried out in any suitable apparatus, for example, those of the pneumatic type such as the calow cell, or those where the air is incorporated with the mixture by agitation such as the Janney apparatus, or the like.

It is of advantage in many cases, as with certain copper ores, to subject the ore pulp to the action of an amount of alkali sufficient to give it a neutral or alkaline reaction before subjecting it to flotation with the aid of the flotation agents of the present invention. The alkali may be caustic alkali such as caustic soda, or an alkaline salt such as soda ash, or it may be calcium oxide or hydrate.

The amount of flotation agent required to be used in the flotation process will vary, it depending partly on the character and composition of the ore, partly on the particular carbocyclic mercaptan employed, and partly on other factors. With many of these agents, one-fifth to one-half of a pound per ton of dry ore will be sufficient. Larger or smaller amounts than this, however, can be used.

The invention will be further illustrated by the following specific examples, but it will be understood that the invention is not limited thereto. The parts are by weight.

*Example 1.*—500 parts of a copper sulfide ore (of the Inspiration Consolidated Copper Company) assaying 1.49 percent copper was ground in a ball mill with 300 parts water and 0.75 parts hydrated lime (equivalent to 3 pounds hydrated lime per ton of ore) until practically all of the mixture was sufficiently fine to pass a 40 mesh screen. The ground pulp was diluted with sufficient water added to give a pulp containing about 16 percent solids and subjected to flotation in a Janney flotation apparatus, with the addition of a solution containing 0.0625 parts of thiophenol (phenyl mercaptan) dissolved in an equivalent amount of normal caustic soda. After agitating for two or three minutes, a small amount, e. g. 0.02 to 0.04 parts of pine oil was added. A

satisfactory mineral froth was produced. During the next 25 minutes of agitation, an equal amount of pine oil was added or enough to make a total of about 0.04 to 0.08 parts in all, i. e., about one-sixth to one-third pound per ton of ore. Mechanical agitation of the pulp was continued for about 5 minutes after all of the pine oil had been added. 58 parts of a concentrate assaying 11.65 percent copper was obtained. A recovery of 92.3 percent of the copper was therefore obtained in the concentrate. The tailings assayed 0.13 percent copper. It will be noted that the equivalent of 8.45 tons of ore were required to give 1 ton of concentrate.

15 In a similar test when using 500 parts of another copper ore (of the Miami Copper Company) assaying 1.21 percent copper and the same amount of thiophenol, there was obtained 22 parts of concentrate assaying 21.1 percent copper which is a recovery of 76.8 percent. The tailings assayed 0.29 percent copper. In this test, the equivalent of 22.7 tons of ore gave 1 ton of concentrate.

Example 2.—500 parts of a copper sulfide ore (of the Miami Copper Company) assaying 1.21 percent copper was treated as described in Example 1 except that 0.0625 parts para-thiocresol (equivalent to one-quarter pound per ton of ore) was used in place of 0.0625 parts of thiophenol. 30 21.8 parts of concentrate assaying 21 percent copper was obtained. This is a recovery in the concentrate of 75.7 percent copper. The tailings assayed 0.31 percent copper. In this example the equivalent of 22.8 tons of ore gave 1 ton of concentrate.

35 In another test when using 500 parts of an ore (of the Inspiration Copper Company) assaying 1.25 percent copper and 0.0625 grams para-thiocresol, but otherwise treated as in Example 1, there was obtained 47.7 parts of concentrate assaying 12.47 percent copper which is a recovery of 88 percent. The tailings assayed 0.18 percent copper. In this test, the equivalent of 10.5 tons of ore gave 1 ton of concentrate.

40 Example 3.—500 parts of a copper sulfide ore (of the Miami Copper Company) assaying 1.25 percent copper was treated as described in Example 1 except that 0.0625 parts beta-thionaphthol (2-mercapto-naphthalene) was used in place of 0.0625 parts of thiophenol. 20.8 parts of concentrate assaying 22.2 percent copper was obtained which is a recovery of 74.1 percent. The tailings assayed 0.34 percent copper. In this example, the equivalent of 23.3 tons ore gave 1 ton of concentrate.

45 Example 4.—500 parts of ore (of the Inspiration Copper Company) assaying 1.47 percent copper was treated as described in Example 1 except that 0.0625 parts of 2-mercapto-anthraquinone was used in place of the 0.0625 parts thiophenol. 51 parts of concentrate assaying 9.9 percent copper was obtained. This is a recovery of 71.5 percent. In this example, the equivalent of 9.45 tons of ore gave 1 ton concentrate. The 50 concentrates obtained in the above examples were so-called "rough" concentrates, that is, they were concentrates which were not "cleaned" by re-treatment or re-flotation.

55 In carrying out the process, the flotation agent can be used in the dry form, if desired; or it can be added to and ground with the ore. It may also be used in conjunction with other frothing agents or with other flotation agents, or with both. In general, it is preferably employed in 60 solution in caustic alkali but its salts, particu-

larly the sodium, potassium or ammonia salts, or salts of organic bases, may also be employed.

It will thus be seen that the present invention utilizes as flotation agents in the separation of minerals and the concentration of ores the nitrogen-free aromatic carbocyclic mercaptan bodies, substances or compounds; that said flotation agents may be incorporated in or with the ore in any suitable or well-known manner; that they may be used in conjunction with other flotation agents or with frothing agents or with both; and that they may be added in the dry state in the free condition or as salts, or in solution, suspension or dispersion in any suitable solvent or medium.

90 The present invention is of more or less general application to the treatment of various kinds of mineral mixtures, both natural and artificial, which are amenable to concentration by flotation processes.

95 It will be further understood that the invention is not limited to the use of the particular agents or ingredients mentioned as examples and that other agents of the class mentioned can be used.

100 In the claims, it will be understood that the expression "nitrogen-free aromatic carbocyclic mercaptan containing not more than fourteen R-carbon atoms in the carbocyclic nucleus" comprehends the nitrogen-free mercaptans of 105 the benzene series (which has six R-carbon atoms), of the naphthalene series (which has ten R-carbon atoms), and the anthracene series (which has fourteen R-carbon atoms). It will be further understood that the expression "hydroxyl group" signifies and includes the hydroxyl group as well as groups or radicals which contain a hydroxyl group, e. g., OH, SO<sub>2</sub>OH, COOH, etc.

We claim:

1. In effecting the concentration of minerals, 115 the process which comprises mixing with the mineral pulp a flotation agent in which there is predominantly present a nitrogen-free aromatic carbocyclic mercaptan body, and subjecting the resulting mixture to a froth flotation operation. 120

2. In effecting the concentration of minerals, the process which comprises subjecting the mineral pulp to a froth flotation operation in the presence of a flotation agent in which there is predominantly present a nitrogen-free thiophe- 125 nol body of the benzene series.

3. In effecting the concentration of minerals the process which comprises subjecting the mineral pulp to a froth flotation operation in the presence of a flotation agent in which there is 130 predominantly present an aromatic nitrogen-free mercaptan, a mercapto group being attached to a carbon atom which is a ring-member of an aromatic nucleus of a carbocyclic series.

4. In effecting the concentration of minerals, 135 the process which comprises subjecting the mineral pulp to a froth flotation operation in the presence of a flotation agent in which there is predominantly present a nitrogen-free aromatic carbocyclic mercaptan embodying within its 140 composition the following atomic grouping:



5. In effecting the concentration of minerals, 145 the process which comprises incorporating with a mineral pulp a flotation agent consisting essentially of a nitrogen-free aromatic carbocyclic mercaptan containing not more than fourteen R-carbon atoms in the carbocyclic nucleus, and 150

- subjecting the resulting mixture to a froth flotation operation.
6. In effecting the concentration of minerals, the process which comprises incorporating with a mineral pulp a flotation agent consisting essentially of a nitrogen-free aromatic carbocyclic mercaptan containing not more than ten R-carbon atoms in the carbocyclic nucleus, and subjecting the resulting mixture to a froth flotation operation.
7. In effecting the concentration of minerals, the process which comprises incorporating with a mineral pulp a flotation agent consisting essentially of a nitrogen-free aromatic carbocyclic mercaptan containing not more than six R-carbon atoms in the carbocyclic nucleus, and subjecting the resulting mixture to a froth flotation operation.
8. In effecting the concentration of minerals, the process which comprises mixing with the mineral pulp a nitrogen-free aromatic carbocyclic mercaptan, having in its composition a double bond adjacent to the grouping C—SH, in the proportions of about one-fifth to about one-half pound of mercaptan per ton of dry mineral, and subjecting the resulting mixture to a froth flotation operation.
9. In effecting the concentration of minerals, the process which comprises mixing with the mineral pulp a flotation agent consisting essentially of an aromatic carbocyclic mercaptan which, besides the mercapto group, contains only carbon and hydrogen in its composition, and in which the mercapto group is attached to a nuclear carbon atom, and subjecting the resulting mixture to a froth flotation operation.
10. In effecting the concentration of minerals, the process which comprises mixing with the mineral pulp an aromatic carbocyclic mercaptan of the benzene series which, besides the mercapto group, contains only carbon and hydrogen in its composition, and in which the mercapto group is attached to a nuclear carbon atom, in the proportions of about one-fifth to about one-half pound of mercaptan per ton of dry mineral, and subjecting the resulting mixture to a froth flotation operation.
11. In effecting the concentration of copper sulfide ores, the process which comprises mixing with a pulp of the ore a flotation agent consisting essentially of phenyl mercaptan, and subjecting the resulting mixture to a froth flotation operation.
12. In effecting the concentration of copper sulfide ores, the process which comprises mixing with a pulp of the ore a flotation agent consisting essentially of para-thiocresol, and subjecting the resulting mixture to a froth flotation operation.
- FREDERICK G. MOSES.  
RAYMOND W. HESS.  
ROBERT L. PERKINS.
- 105
- 35 110
- 40 115
- 45 120
- 50 125
- 55 130
- 60 135
- 65 140
- 70 145
- 75 150